

Feb. 28, 1933.

J. A. SWEENEY

1,899,736

OPHTHALMIC MOUNTING AND METHOD OF MAKING THE SAME

Original Filed March 9, 1929



Fig. 1



Fig. 2



Fig. 3

Fig. 4



Fig. 5

Fig. 6

Inventor  
James A. Sweeney  
By David Rines  
Attorney

## UNITED STATES PATENT OFFICE

JAMES AUGUSTUS SWEENEY, OF PROVIDENCE, RHODE ISLAND

## OPHTHALMIC MOUNTING AND METHOD OF MAKING THE SAME

Application filed March 9, 1929, Serial No. 345,862. Renewed July 18, 1932.

The present invention relates to ophthalmic mountings and to methods of making the same.

As ophthalmic mountings are conspicuously worn upon the face, they should be beautiful, else many persons will not wear them at all. Metal mountings produce more or less of an ugly effect as they tend to give the countenance a pallid appearance. Some persons have, therefore, turned, for many years, to tortoise shell, celluloid and other compositions. But as metal mountings have many advantages not possessed by such substitutes, attempts have been made, at various times, to cause the metal mountings to return to favor. Thus, optical manufacturers have, of recent years, tried to please the eye by building metal mountings in fantastic shapes; but such shapes can not be more than a passing fancy.

Among the objects of the present invention are to provide a new and improved ophthalmic mounting of pleasing appearance, and a novel method of manufacturing the same. Other and further objects will be explained hereinafter and will be particularly pointed out in the appended claims.

The nature and the objects of the invention will be explained in connection with the accompanying drawing, in which Fig. 1 is an elevation illustrating a step in the manufacture of an ophthalmic-mounting lens rim; Fig. 2 is an enlarged fragmentary section of the same, taken upon the line 2-2 of Fig. 3; Fig. 3 is a similar section taken upon the line 3-3 of Fig. 2; Fig. 4 illustrates a further step in the manufacture; and Figs. 5 and 6 are, respectively, a front and a side elevation of a preferred embodiment of the ophthalmic mounting of the present invention.

The improved ophthalmic mounting illustrated comprises two lens-holding rims 2 connected by a bridge 4 and having temples 6 and nose guards 8. To beautify the mounting, the rims 2 are provided with peripheral stripes 10; the bridge 4 with a longitudinal stripe 12; and the forward portions of the temples 6, near where they are pivoted to the rims 2, with longitudinal stripes 14. These stripes 10, 12 and 14, as will hereinafter appear, are preferably constituted of enamel.

Enamel, as is well known, presents a hard surface that is easily liable to crack. This is particularly to be guarded against in connection with ophthalmic mountings, as they require bending adjustments to fit the patient originally and after they get out of shape, and they are, furthermore, flexed back and forth many times a day when put on, and taken off, the face. Thus, the bridge 4 must be bent in and out to adjust for pupillary distance, and the rims 2 must be opened and closed to insert and remove lenses, and must be bent to fit different sizes and shapes of lenses. The grasping by the hands of the rear curved portions of the temples, that are adapted to hold the mounting on the wearer's face, cause repeated bendings and flexings in the forward parts of the temples and also in the bridge 4 and the rims 2. Such adjustment and flexing of the ophthalmic mounting necessarily introduces stresses and strains in the enamel. Not only that, but because of such constant use of this character, the enamel has a tendency to peel off the mounting, even without cracking. Optical manufacturers and opticians, furthermore, as well as individual wearers of the mountings, have a habit of dipping the mountings into cleansing liquids, not merely for the purpose of brightening up the metal of the mounting (to remove finger marks of shop workmen, and opticians, and other foreign dust substances), but even more often as preparatory to wiping the lenses. The enamel must, of course, be of a character to resist the chemical attacks of such cleansing liquids. Ordinary enamels, finally, require long baking processes to cause them to harden and adhere, and such baking processes are out of the question for the manufacture of ophthalmic mountings. It will readily be appreciated, therefore, that to provide an ophthalmic mounting of the above-described character involves great difficulties.

According to the present invention, the ophthalmic-mounting part that is to receive the enamel is first provided with a shallow, enamel-holding channel or groove 16, preferably rectangular-shaped in cross section, as illustrated. The channel or groove 16 may

be three millimeters deep. The channel may be made in the lens-holding rims 2 by means of rolls 18 and 20 so shaped that, when the metal wire is drawn between them, they shall 5 form therein, at a single operation, both the lens-holding groove 22 and the groove or channel 16. The bridge 4 may have its enamel-receiving groove produced in similar fashion. Corresponding externally-disposed 10 longitudinal grooves may be formed in the forward portions of the temples 6, or the temples 6 may be formed by means of dies. The bottom of the channel or groove is provided with small enamel-holding projections, 15 shown at 24. The projections 24 may be of any suitable shape, but practice has demonstrated that best results are obtained when these projections produce a kind of matted surface over the bottom of the channel or groove. 20 The matted construction may, of course, result from suitably shaping the rolls or dies, as shown at 26, so that the projections 24 may be formed simultaneously with the formation of the enamel-receiving channel or 25 groove. In this manner, the channel or groove will be enabled to hold a correspondingly shaped layer of enamel securely between its walls 28 and 30 interlocked with the projections 24. 30 The next step is to cleanse the mounting thoroughly, as by dipping it in a solution of carbon tetrachloride, to remove the grease from the mounting, after the mounting is polished, as on a polishing wheel, with rouge. 35 A thin layer or coating of enamel is then applied. This may be done by progressively moving a brush, ruling pen, draw pen, or any other suitable instrument 32, as illustrated in Fig. 4, continuously over successive portions 40 of the channel or groove, until a continuous layer of the enamel has been applied to the whole length of the groove. The enamel is then allowed to dry or harden in its groove. If the enamel is constituted of the proper in- 45 gredients, and in suitable proportions, the enamel will dry quickly without any baking whatever, will flex readily without cracking, and will resist the chemical attacks of all ordinary cleansing washes. Indeed, if the 50 enamel is of the right consistency, it will be found to dry sufficiently well to adhere to the matted surface 24 almost as soon as it is applied, and before the mounting has left the operator's hands. This is particularly valuable 55 for use with ophthalmic mountings, as it permits applying the enamel to the bridge 4 and to the periphery of the whole lens-holding rim 2 in practically a single operation, and without waiting for the one half of the 60 rim to become baked before it is turned upside down to enable application of the enamel to the other half of the rim, without danger of the enamel flowing out of its groove during the process. The matted surface 24 helps 65 hold the enamel in place until it quickly

dries; on a smooth, glassy surface, the enamel would have a tendency to flow downward before it could have a chance to dry. A single layer or coating of the enamel, if of the right consistency, is all that needs to be applied, 70 though several layers could, of course, be used, if desired, each layer being allowed to dry before the next layer is applied. This, however, would involve an unnecessary waste of time. 75

The following ingredients will produce a soft, bendable, non-cracking, quick-drying enamel that satisfies all the above requirements:

Substantially equal proportions of wood 80 charcoal and gum resin are ground and mixed together, and linseed oil and turpentine are added. When the enamel is ready to use, 20% ether is added to 80% of the composition. The liquid should be of consistency such as to make it possible to use one of the before-mentioned instruments 32. The charcoal and gum resin may each form 30% of the resulting enamel, and the linseed oil and turpentine each 10%. 90

The overflow enamel may be removed by wiping with a piece of chamois immersed in butyric ether. The enamel is then allowed to harden, by permitting the ether solvent to evaporate. The final step is to burnish off the excess enamel, after which the enamel is glossed upon a polishing wheel, as with black rouge, and washed. The glossing operation may safely be performed within half an hour 95 of the application of the enamel. 100

As before stated, there is no heating or baking and no tying up of production for days at a time on account thereof. Indeed, an enamel that would require baking would probably be brittle, and so unusable upon 105 bendable ophthalmic mountings.

The resulting product will stand up against all ordinary wear, without the enamel disappearing in use, and irrespective of bending and flexing. 110

The enamel may be black or colored or transparent. Thus, it may be of the same color as the color of the metal frame, and transparent, in which event the bottom of the enamel-receiving channel or groove may be 115 engraved or otherwise ornamented to present a pleasing appearance through the enamel.

Modifications will occur to persons skilled in the art, and all such are considered to fall within the spirit and scope of the invention, 120 as defined in the appended claims.

What is claimed is:

1. An ophthalmic mounting comprising a bendable member having a groove rectangular in cross section, and a correspondingly shaped bendable layer of enamel in the groove, the enamel being constituted of charcoal and gum resin. 125

2. A spectacle temple having a forward portion at which it is adapted to be hinged 130

to a spectacle frame and a rear curved portion adapted to engage the wearer's body to hold the spectacles in place, the forward portion of the temple being bendable and being 5 exteriorly provided with a longitudinally disposed groove, and a correspondingly bendable layer of enamel longitudinally disposed in the groove.

3. A method of making an ophthalmic 10 mounting that comprises providing an ophthalmic-mounting member with a groove, progressively applying an enamel of charcoal and gum resin continuously to successive portions of the groove until a continuous layer of the enamel has been applied to the groove, and permitting the layer of the 15 enamel to harden in the groove.

In testimony whereof, I have hereunto 20 subscribed my name.

JAMES A. SWEENEY.

25

30

35

40

45

50

55

60

65